

## UNITED STATES PATENT OFFICE

2,186,685

## PHOTOGRAPHIC COLOR PICTURE

Wilhelm Schneider and Hans Loleit, Dessau, Germany, assignors, by mesne assignments, to Agfa Ansco Corporation, Binghamton, N. Y., a corporation of Delaware

No Drawing. Application April 3, 1939, Serial No. 265,759. In Germany April 9, 1938

8 Claims. (Cl. 95—6)

Our present invention relates to the manufacture of photographic color pictures.

In a process for producing color photographic pictures with aid of color development there are used as dyestuff formers compounds which during the development with a developer containing a free amino-group, for instance para-phenylenediamine or para-aminophenol, yield a dyestuff image on the silver image. For obtaining blue dyestuffs there have hitherto been used by preference phenols and naphthols and derivatives thereof. These dyestuff formers yield during development blue to blue-green quinoneimine dyestuffs.

15 Our present invention has for one object to provide a process of making blue-violet and red-violet photographic pictures.

Another object of our invention is to provide a process of producing such pictures wherein 20 there are used as dyestuff formers compounds of the general formula



25 in which

R is hydrogen, alkyl, aryl, aralkyl, carboxyl or an esterified or aminated carboxyl group and 30 X is vinylene, substituted vinylene, phenylene or substituted phenylene.

A further object of this invention is the provision of a dyestuff forming developer which contains such dyestuff former.

35 Other objects of our invention will appear more in detail hereinafter.

Compounds of this kind are, for example, 2-methyl-indole, 2,5-dimethylindole, 4-phenyl-2-methyl-pyrrole-3-carboxylic acid ethyl ester, 2-methyl-pyrrole-3-carboxylic acid ethyl ester, 2-methyl-pyrrole.

40 These dyestuff components may be added to the developer or to the emulsion. When the component is added to the developing solution it is recommended that it should first be dissolved in an organic solvent, for instance alcohol or acetone, and this solution should be added to the developer.

45 When the dyestuff former is to be added to the photographic silver halide emulsion those formers are especially suitable which, owing to the introduction of special groups, are fast to diffusion with respect to the binding agent of the emulsion. This expedient is especially of importance in the case of dyestuff formers which

are to be used in the production of photographic multi-layer material. The introduction of groups which impart fastness to diffusion has been described in the U. S. Patents 2,179,238, 2,178,612 and 2,179,244 and U. S. patent applications Ser. Nos. 94,340 filed August 5, 1936, 158,860 filed August 13, 1937, 159,518 filed August 17, 1937, 164,499 filed September 18, 1937, 166,832 filed October 1, 1937, 171,705 filed October 29, 1937, 175,285 filed November 18, 1937, 10 176,058 filed November 23, 1937, 191,952 filed February 23, 1938, and in the British patent specification No. 488,048. Said last named U. S. application describes components which contain in addition to a group rendering the component 15 fast to diffusion a solubilizing group such as a carboxy group. The components are prepared by reacting the internal anhydride of a polybasic organic acid, such as the anhydrides of maleic acid, succinic acid, pyrotartaric acid and 20 the like containing for example a long aliphatic chain, i. e. of at least 5 carbon atoms such as octadecylene, isodecylene, iso-nonylene and the like with a color former containing a reactive group such as an amino- or hydroxy group. The ring 25 of the anhydride is thereby split in such a manner that one CO-group unites with the reactive group and the other forms a carboxy group. As the color former there may be used p-amino-aceto-acetic anilide, 4-amino-1-phenyl-3-methyl-5-pyrazolone, 1-amino-5-naphthol and the like. 30 As the anhydride there may be used octadecylene succinic acid anhydride  $\alpha$ -dodecyl- $\alpha$ -hexahydrobenzene-pyro-tartaric acid anhydride and the like. It has been explained in the said application 35 that the radicles which impart fastness to diffusion may be introduced in a manner in itself known, for example by way of amino-, hydroxy- or carboxyl-groups, with the formation of an acid amide or an ester. For example, it is possible 40 to cause 2-methyl-pyrrole-3-carboxylic acid ethyl ester to react with undecylamine. It is also possible to unite the radicle which imparts fastness to diffusion directly to the nitrogen atom without interposition of an acid group or directly 45 to the benzene nucleus. Silver halide emulsion layers comprising such dyestuff components may be applied singly or together with other layers on one or both sides of a carrier to produce a multi-layer material in which the layers are 50 sensitized for different regions of the spectrum. It is also possible to distribute the particles of emulsion containing various dyestuff formers on a carrier. With the aid of this latter material screen pictures may be produced.

5

15

20

25

30

35

40

45

50

55

The silver halide emulsion layers containing the dyestuff formers may be united with other layers generally used in the production of photographic materials, for example filter layers, anti-halation layers, matting layers, backing layers. They may also be combined with photographic layers in which color pictures are to be produced by any other process for instance by the silver bleaching out dyestuff process or the toning process. As binding agent for the photographic emulsions gelatin or any other colloid usual in photographic practice may be used.

The following examples illustrate the invention:

15 *Example 1.*—An exposed silver halide emulsion layer is developed with a developer of the following composition: 1.6 grams 2-methyl-pyrrole-3-carboxylic acid ethyl ester of the formula



|    |                                        |       |      |
|----|----------------------------------------|-------|------|
| 25 | Methanol                               | cc    | 60   |
|    | Para-diethylaminoaniline hydrochloride | grams | 2    |
|    | Crystallized sodium carbonate          | do    | 50   |
|    | Anhydrous sodium sulfite               | do    | 2    |
| 30 | Potassium bromide                      | do    | 0.2  |
|    | Water                                  | cc    | 1000 |

After the silver has been dissolved there remains a blue-violet dyestuff image.

35 *Example 2.*—An exposed silver halide emulsion layer is developed with a developer of the following composition: 2.3 grams 2-methyl-4-phenyl-pyrrole-3-carboxylic acid ethyl ester of the formula



|    |                                        |       |      |
|----|----------------------------------------|-------|------|
| 45 | Methanol                               | cc    | 100  |
|    | Para-diethylaminoaniline hydrochloride | grams | 2    |
|    | Crystallized sodium carbonate          | do    | 50   |
|    | Anhydrous sodium sulfite               | do    | 2    |
| 50 | Potassium bromide                      | do    | 0.2  |
|    | Water                                  | cc    | 1000 |

After dissolving the silver there remains a blue-violet dyestuff image.

55 *Example 3.*—An exposed silver halide emulsion layer is developed with a developer of the following composition:

|                                        |       |     |
|----------------------------------------|-------|-----|
| 2-methylindole                         | grams | 1.3 |
| Methanol                               | cc    | 400 |
| Para-diethylaminoaniline hydrochloride | grams | 2   |
| Crystallized sodium carbonate          | do    | 50  |
| Anhydrous sodium sulfite               | do    | 2   |
| Potassium bromide                      | do    | 0.2 |
| Water                                  | cc    | 600 |

65 After dissolving the silver there remains a blue-violet dyestuff image.

70 *Example 4.*—3 grams of 2-methyl-indole are dissolved in 50 cc. of methanol and the solution is added to 1 kilo of a silver halide emulsion. A layer cast from this emulsion yields after exposure and development with para-diethylaminoaniline a violet dyestuff image.

75 *Example 5.*—0.5 gram of 2.4-dimethyl-3-ethyl-pyrrole is dissolved in a sufficient amount of

methanol (about 20 cc.) and added to 100 cc. of a solution of the following composition:

|                                       |       |      |
|---------------------------------------|-------|------|
| Diethylphenylenediamine hydrochloride | grams | 2.5  |
| Anhydrous sodium sulfite              | do    | 0.5  |
| Potassium bromide                     | do    | 2.5  |
| Potassium carbonate                   | do    | 75   |
| Water                                 | do    | 1000 |

10 The exposed film is developed for eight minutes in this solution which, if necessary, has been clarified by adding methanol and filtered. After fixing and bleaching by means of potassium ferricyanide a violettish picture is obtained.

15 *Example 6.*—0.5 gram of 2.5-dimethylindole is dissolved in methanol and added to 100 cc. of a solution having the composition described in Example 5. The film is developed and worked up in the same manner as mentioned in Example 5. A red-violet picture is obtained.

20 *Example 7.*—0.5 gram of 2-methyl-4-phenyl-3-acetylpyrrole is dissolved in methanol and added to 100 cc. of a solution having the composition described in Example 5. The film is developed and worked up in the same manner as mentioned in Example 5. A blue picture is obtained.

25 *Example 8.*—0.5 gram of 2-methyl-4-phenyl-3-cinnamoylpyrrole is dissolved in methanol and added to 100 cc. of a solution having the composition described in Example 5. The film is developed and worked up in the same manner as mentioned in Example 5. A blue-violet picture is obtained.

30 *Example 9.*—0.5 gram of 2-methyl-4-phenyl-pyrrole-3-carboxylic acid is dissolved in methanol and added to 100 cc. of a solution having the composition described in Example 5. The film is developed and worked up in the same manner as mentioned in Example 5. A blue-violet picture is obtained.

35 *Example 10.*—0.5 gram of 2.4-dimethyl-3-acetylpyrrole is dissolved in methanol and added to 100 cc. of a solution having the composition described in Example 5. The film is developed and worked up in the same manner as mentioned in Example 5. A blue-violet picture is obtained.

40 *Example 11.*—0.5 gram of 2-methyl-4-phenyl-3-benzoylpyrrole is dissolved in methanol and added to 100 cc. of a solution having the composition described in Example 5. The film is developed and worked up in the same manner as mentioned in Example 5. A blue-violet picture is obtained.

45 *Example 12.*—3 grams of the condensation product from 2 mols of 2-methyl-4-phenyl-3-acetylpyrrole and 1 mol of diphenyl-dialdehyde is dissolved in 60 cc. of acetone. The solution is added to 1 kilo of a silver halide gelatin emulsion. The emulsion is then cast to form a layer of a photographic multi-layer material. A blue-violet picture is obtained in this layer.

55 *Example 13.*—2-methyl-4-phenyl-3-acetylpyrrole is condensed with m-nitrobenzaldehyde and after the nitro-group has been reduced to an amino-group the reaction product is further condensed with palmitic acid chloride in pyridine. 3 grams of the product thus obtained are dissolved in 60 cc. of acetone. The solution is added to 1 kilo of a silver halide gelatin emulsion. The emulsion may be used for the manufacture of a multi-layer material. A blue-violet picture is obtained in this emulsion layer.

We claim:

1. In a process of producing photographic

color pictures by dyestuff forming development, the step which comprises causing as the dyestuff former a compound of the general formula



wherein

10 R is a member selected from the class consisting of hydrogen, alkyl, aryl, aralkyl, carboxyl, esterified carboxyl, and aminated carboxyl and

15 X is a member selected from the class consisting of vinylene, substituted vinylene, phenylene, and substituted phenylene,

to react with the oxidation product of an aromatic developer.

2. In a process of producing photographic color pictures by dyestuff forming development, the step which comprises developing the exposed photographic silver halide emulsion with an aromatic amino developer containing as the dyestuff former a compound of the general formula



30 wherein

R is a member selected from the class consisting of hydrogen, alkyl, aryl, aralkyl, carboxyl, esterified carboxyl, and aminated carboxyl and

35 X is a member selected from the class consisting of vinylene, substituted vinylene, phenylene, and substituted phenylene.

3. In a process of producing photographic color pictures by dyestuff forming development, the step which comprises exposing a photographic silver halide emulsion containing as the dyestuff former a compound of the general formula



wherein

50 R is a member selected from the class consisting of hydrogen, alkyl, aryl, aralkyl, carboxyl, esterified carboxyl, and aminated carboxyl and

55 X is a member selected from the class consisting of vinylene, substituted vinylene, phenylene, and substituted phenylene,

said compound containing a radicle imparting thereto fastness to diffusion with respect to the

binding agent of said emulsion, and developing said emulsion with an aromatic amino developer.

4. Silver halide emulsion for color photography comprising a compound of the general formula



wherein

10 R is a member selected from the class consisting of hydrogen, alkyl, aryl, aralkyl, carboxyl, esterified carboxyl, and aminated carboxyl and

15 X is a member selected from the class consisting of vinylene, substituted vinylene, phenylene, and substituted phenylene,

said compound containing a radicle imparting thereto fastness to diffusion with respect to the binding agent of said emulsion.

20 5. A dyestuff forming developer comprising an aqueous solution containing an aromatic amino developing agent and a compound of the general formula



wherein

30 R is a member selected from the class consisting of hydrogen, alkyl, aryl, aralkyl, carboxyl, esterified carboxyl, and aminated carboxyl and

35 X is a member selected from the class consisting of vinylene, substituted vinylene, phenylene, and substituted phenylene.

3. The silver halide emulsion as defined in claim 4, wherein the radicle imparting fastness to diffusion is linked to the compound by a linkage selected from the class consisting of a direct carbon to carbon linkage, an ester linkage, an acid amide linkage and a direct nitrogen to carbon linkage.

6. A silver halide emulsion for color photography containing as the color forming component the reaction product of 2-methyl-pyrrole-3-carboxylic acid ethyl ester with undecylamine.

7. A silver halide emulsion for color photography containing as the color forming component a 2-methyl-indole substituted in 5-position by a member of the group consisting of methyl and hydrogen, said indole having attached thereto a radicle which renders the indole fast to diffusion with respect to the binding agent of the emulsion.

WILHELM SCHNEIDER.  
HANS LOLEIT.